

## UNITED STATES PATENT OFFICE

HENRY DREYFUS, OF LONDON, ENGLAND

## MANUFACTURE OF ARTIFICIAL SILK, ARTIFICIAL HORSEHAIR AND LIKE PRODUCTS

No Drawing. Original application filed June 28, 1923, Serial No. 648,350, and in Great Britain August 11, 1922. Divided and this application filed April 5, 1928. Serial No. 267,808.

This application is a divisional application from my U. S. application Serial No. 648,350 which eventuated into Patent No. 1,688,531, granted October 23, 1928.

5 This invention relates to the manufacture of artificial silk, artificial horsehair or like threads or filaments from solutions of cellulose acetate in particular, but applies also to their production from other solutions of esters of cellulose or of ethers of cellulose such for example as ethyl-, methyl- or benzyl cellulose, or from mixtures of any of such cellulose derivatives, all of which cellulose derivatives are hereinafter in the claims referred to as organic substitution derivatives of cellulose. The invention solely concerns processes in which the artificial threads or filaments are produced by the dry or evaporative method of formation, that is to say by 10 extruding a solution of the cellulose derivative or derivatives in or containing a volatile or vaporizable solvent or solvents, through jets or spinnerets into a heated or other atmosphere in which the filaments or threads 15 solidify by evaporation of solvent. In particular the invention relates to the manufacture of threads, filaments or the like from cellulose acetate solutions by dry or evaporative spinning.

20 In the manufacture of artificial threads or filaments from solutions of cellulose acetate or other cellulose esters or ethers such as referred to by the evaporative method, it is usual to employ spinning solutions of relatively low concentration, containing not more than about 16% of the cellulose derivative or derivatives in the solvent or solvents used.

It has now been found that by employing 25 for the dry or evaporative spinning solutions of substantially higher concentrations, containing more than 20% of the cellulose derivative or derivatives, and especially in the case of cellulose acetate solutions, artificial threads or filaments of improved 30 quality can be obtained, possessing greater mechanical strength and rounder section, and showing much less tendency to crinkle or turn woolly in appearance under the action of very hot or boiling water, than is the case with dry-spun artificial threads or

filaments, made from the less concentrated solutions previously employed. It is moreover found that, especially in the case of cellulose acetate, the employment of solutions of high concentrations as referred to has 55 the further advantage of obviating or greatly reducing what may be called "glitter" of the threads, filaments or the like, that is to say, a glittering or scintillating effect which is sometimes possessed by filaments or 60 threads formed by dry or evaporative spinning from solutions of the relatively low concentration usually employed, and possibly due to the sectional configuration of the filaments resulting from the spinning of such 65 solutions, by the dry or evaporative method of formation. This "glitter" effect or glitter-producing structure of the filaments or the like can in some cases be a disadvantage. For example, in cases where goods in hank, 70 woven or knitted fabric or other form, made with threads showing such glitter effect are dyed in black or dark colours, it is sometimes found that the dyed goods give an impression as if the artificial silk is dyed only partially 75 or not deep enough or that they have a worn appearance, this being more especially seen in fabrics. Each per cent increase in the concentration of the solutions of the cellulose acetate or other cellulose derivatives over 80 85 and above 20% is accompanied by a great increase in the viscosity of the spinning solutions and in the strength of the filaments or threads obtained. Moreover, at a concentration of about 21%, glitterless filaments are obtainable. At a concentration of 22% the roundness and strength of the filaments is still more marked.

By forming the dry spun threads, filaments or the like from cellulose acetate solutions, for 90 example, of high concentrations such as before referred to, namely 21 or 22 to 25%, it will be seen that the filaments or threads are stronger than those made from solutions of the usual low concentrations, not so liable to crinkle or turn woolly as a result of the action of hot water, and moreover that "glitter" or glitter-producing structure is obviated or greatly reduced, with its tendency to 95 give on dyed goods, and especially goods dyed 100

in black or dark colours, the appearance before referred to.

The following are two examples of spinning solutions which may be employed according to the invention, it being understood that these are given only by way of illustration and that other solvents or solvent mixtures may be employed and that the concentrations can be varied without departing from the invention.

*Example 1*

Cellulose acetate is dissolved in acetone in quantity to give a solution containing between 21 and 25% cellulose acetate.

*Example 2*

Cellulose acetate is dissolved in acetone containing about 5 to 10% of alcohol and about 5% of water, in a quantity to give a solution containing between 22 and 25% of cellulose acetate in the solvent mixture.

The solutions are dry spun in the known way by extrusion through spinnerets into a heated atmosphere.

While my invention relates especially to the manufacture of artificial threads, filaments or the like from cellulose acetate solutions by the dry or evaporative method it is also applicable to their production by the dry or evaporative method from solutions of other cellulose esters or ethers or mixtures of cellulose esters or/and ethers.

What I claim and desire to secure by Letters Patent is:—

1. Process for the manufacture of artificial filaments and threads, characterized in that the same are dry spun from concentrated solutions of organic substitution derivatives of cellulose containing at least 21 and less than 25% of the cellulose derivative.

2. Process for the manufacture of artificial filaments and threads, characterized in that the same are dry spun from concentrated solution of organic substitution derivatives of cellulose containing at least 22 and less than 25% of the cellulose derivative.

3. Process for the manufacture of artificial filaments and threads, characterized in that the same are dry spun from concentrated solutions of cellulose acetate containing at least 21 and less than 25% of cellulose acetate.

4. Process for the manufacture of artificial filaments and threads, characterized in that the same are dry spun from concentrated solutions of cellulose acetate containing at least 22 and less than 25% of cellulose acetate.

In testimony whereof I have hereunto subscribed my name.

60 HENRY DREYFUS.